

[54] **LIGHT-SENSITIVE MATERIAL  
CONTAINING A POLYHALOGENATED  
HYDROCARBON, AN  
N-VINYLCARBAZOLE, AND A  
FURFURYLIDENE COMPOUND AS AN  
IMAGE ENHANCER AND STABILIZER**

[75] Inventors: **Hiroshi Yamashita; Nobuyoshi  
Sekikawa**, both of Asaka, Japan

[73] Assignee: **Fuji Photo Film Co., Ltd.,  
Kanagawa, Japan**

[22] Filed: **Dec. 29, 1971**

[21] Appl. No.: **213,538**

[30] **Foreign Application Priority Data**

Dec. 29, 1970 Japan..... 45/121448

[52] **U.S. Cl..... 96/90 R, 96/115 P**

[51] **Int. Cl..... G03c 1/52, G03c 1/68**

[58] **Field of Search .....** 96/90 R, 88, 115 P

[56] **References Cited**

**UNITED STATES PATENTS**

|           |         |                   |          |
|-----------|---------|-------------------|----------|
| 3,394,395 | 1/1968  | Mattor et al..... | 96/90 R  |
| 3,544,322 | 12/1970 | Yamada.....       | 96/48 R  |
| 3,697,276 | 10/1972 | Lewis et al.....  | 96/48 HD |

*Primary Examiner*—Norman G. Torchin

*Assistant Examiner*—Won H. Louie, Jr.

*Attorney*—Richard C. Sughrue et al.

[57] **ABSTRACT**

A non-silver halide light-sensitive material for dry processing containing (a) polyhalogenated hydrocarbon, (b) N-vinylcarbazole, (c) a furfurylidene compound and optionally at least one of the following; hydroquinone, resorcinol, derivatives thereof, a dye or dye bases.

**14 Claims, No Drawings**

**LIGHT-SENSITIVE MATERIAL CONTAINING A POLYHALOGENATED HYDROCARBON, AN N-VINYLCARBAZOLE, AND A FURFURYLIDENE COMPOUND AS AN IMAGE ENHANCER AND STABILIZER**

**DESCRIPTION OF THE PRIOR ART**

There are many patents relating to non-silver halide light-sensitive materials comprising a combination of an organic halogen compound and an aromatic amine, such as the U.S. Pat. Nos. 3,042,515; 3,042,516; 3,042,517; 3,042,518; 3,042,519, etc. The main problem with such elements is how to fix the element, that is, how to increase the stability of the obtained image and how to remove the light sensitivity remaining at unexposed portions. Usually, unexposed portions are desensitized by heating or treating with a solvent after the exposure. Mere heating, however, is not sufficient, and treatment with a solvent requires a long period of time and has defects such as toxicity.

Some attempts have been made to solve these problems. In U.S. Pat. No. 3,082,086 (Japanese Pat. No. 17701/64), a secondary amine is inactivated by the reaction between aromatic amine and carboxylic acid anhydride to remove the remaining light-sensitivity. The anhydride, however, is so liable to be hydrolyzed by moisture in the air that it lacks storage stability.

In Japanese Pat. No. 16,753/70, the remaining light sensitivity is removed by treatment with an aqueous solution containing a reducing heavy metal, a wet processing.

In Japanese Pat. No. 22,941/69, the adduct of a bisulfite and a compound containing a carbonyl group is used for fixing.

Light-sensitive materials comprising carbon tetrabromide and N-vinylcarbazole are described in U.S. Pat. Nos. 3,476,562; 3,503,745, etc. Fixing processes thereof are known, e.g., in U.S. Pat. No. 3,503,742 (Japanese Pat. No. 2,619/68) the unexposed portions are desensitized by treatment with ammonia. However, ammonia is not preferred due to its pungent odor and its toxicity.

In U.S. Pat. No. 3,512,916, fixing is carried out by treatment with an aqueous solution of sodium sulfite, etc., but this is a wet processing and has the defect that treatment requires a long period of time.

The components (a) and (b) are necessary for the combination of the components (a), (b), (e), namely polyhalogenated hydrocarbon, N-vinylcarbazole, and dye or dye base, thus see U.S. Pat. No. 3,503,745. Further, for the combination of the components (a), (b), (d), namely polyhalogenated hydrocarbon, N-vinylcarbazole, and hydroquinone, resorcin or derivatives see U.S. Pat. No. 3,544,322.

**SUMMARY OF THE INVENTION**

The present invention relates to a dry processing non-silver halide light-sensitive material which provides a black stable image and is characterized by the inactivation of unexposed portions by heating. More particularly, it relates to a light-sensitive material having the following composition; (a) polyhalogenated hydrocarbon, (b) N-vinylcarbazole, (c) furfurylidene compound, and optionally at least one of (d) hydroquinone, resorcinol and derivatives thereof and (e) a dye or dye base.

The action of ingredients (a) to (e) in the light-sensitive material is believed to be as follows.

Ingredient (a) is a photo-activator which produces free radicals or ions by the action of light. N-vinylcarbazole (b) reacts with the free radicals or ions produced to develop color. Ingredient (c) is capable of providing a black image which is necessary to obtain a stable image and, at the same time, the resulting image density increases and the light fastness thereof is good. Ingredient (d) has two functions—improving the shelf life of the sensitive material (acting as a stabilizer) and inactivating unexposed portions upon heating to 70°-150° C (acting as a fixing agent). Ingredient (e) has two functions: improving the shelf life and a spectrally sensitizing action.

The present invention includes a fixed process having no defects such as those described above.

**DETAILED DESCRIPTION OF THE INVENTION**

20 The fundamental composition of the light-sensitive material of the present invention is: (a) polyhalogenated hydrocarbon, (b) N-vinylcarbazole, (c) furfurylidene compound, and optionally at least one of (d) hydroquinone, resorcinol and derivatives thereof, and (e) a dye or dye base.

| Components                          | Mixture Ratio | Preferably                            |
|-------------------------------------|---------------|---------------------------------------|
| (b)/(a)                             | 50/1-1/50     | 5/1-1/5                               |
| (b)/(c)                             | 100/1-1/100   | 10/1-1/10                             |
| (b)/(d)                             | 1000/1-1/5    | 200/1-1/2                             |
| (b)/(e)                             | 10/1-1/1      | 10 <sup>3</sup> /1-10 <sup>3</sup> /1 |
| 30 binder/light-sensitive component | 1/100-20/1    | 1/10-5/1                              |

35 N-vinylcarbazole and carbon tetrabromide cause a thermal reaction because they form a charge-transfer complex of 1:1, 2:1, etc., and hence they seem to have a poor storage stability. Therefore, storage stability will be improved by the addition of a substance that prevents such a thermal reaction. It is the ingredient (d) that corresponds to such substance.

40 45 The dye produced by the photochemical reaction between carbon tetrabromide and N-vinylcarbazole is unstable, especially lacking light fastness. For example, in the case of a sensitive material wherein gelatin is used as a binder, there is obtained, immediately after processing, a greenish-blue image with a yellow background, but, in a bright room, the whole turns dark brown, and a brown colored image appears in the background. As is mentioned above, in a light sensitive material comprising carbon tetrabromide and N-vinylcarbazole, there are the two problems of the stability of the image formed and fogging at the unexposed portions. The present invention has solved these problems. The fogging at the unexposed portions supposedly results from the color reaction between N-vinylcarbazole polymer and carbon tetrabromide to add to the reaction between non-reacted materials.

50 55 The formation of the N-vinylcarbazoles is sufficiently contemplated. The molecular weights are supposed about from thousands to scores of thousands.

60 65 It is believed that the fogging at the unexposed portions results from the color reaction between one polyvinylcarbazole and carbon tetrabromide, and the reaction of non-reacted materials, N-vinylcarbazole and carbon tetrabromide.

65 70 It has been found that a black, stable color developed body can be obtained with increased image density by the addition of the ingredient (c) to this system. The

black image can be obtained by dry processing, which will extend the regions of application of such an element. For example, the light-sensitive material of the present invention can be used instead of an usual printing paper comprising silver halide. It has the advantage that the treatment thereof is easy due to the dry processing. Besides, in the case of adding the ingredient (d), apart from acting as a stabilizer, the unexposed portions can be desensitized by heating to 70° - 150°C after imagewise exposure. The temperature range is from 40° - 250°C, preferably from 70°C - 150°C. In addition, the unexposed portions are clear white, and hence fog density is extremely low. When ingredients (c) and (d) are present, a blackish brown image is obtained with a white background. The image formed hardly changes in a bright room.

When the ingredient (e) is added, the sensitive wavelength region is extended to about 700nm.

When a dye base was used, a rise in sensitivity at the intrinsic region was encountered. In a non-sensitized system, the light-sensitive region is up to 480 nm. It was also found that by the addition of the ingredient (e) the storage stability of the sensitive material was remarkably improved.

As the ingredient (a) of the present invention, the following polyhalogenated hydrocarbon can be used:



wherein R represents H, X, COOR', — C(H)<sub>3</sub>—nX<sub>n</sub>, X being Cl, Br or I, R' being H, CH<sub>3</sub> or C<sub>2</sub>H<sub>5</sub> and m and n being 2 or 3.

As ingredient (c), which stabilizes the image formed and increases the density to blacken the image, the following furfurylidene compounds can be used:



wherein X represents nothing,



wherein Y and Y' represent H or alkyl group, or



As the stabilizing and fixing ingredient (d), there can be used hydroquinone, resorcinol and the derivatives thereof, e. g.,



wherein R and R' represent H, an alkyl group of one to six carbon atoms, aryl, hydroxyalkyl, benzoyl, acetyl or



5 , R'' represents H, alkyl, halogen, or alkoxy, and n represents an integer of 1-4.

As the stabilizing and spectrally sensitizing ingredient (e), there can be used dyes or dye bases (which are converted to a dye by oxidation) such as photographic spectral sensitizing dye materials being in a form selected from a dye form or a dye base form, such as anthraquinone dyes, triphenylmethane dyes, xanthene dyes, acridine dyes, azine dyes, thiazine dyes, cyanine dyes, styryl dyes, etc.

Above dyes are as follows: anthraquinone dyes such as alizaline (CI5800), purpurin (CI1037), alizaline cyanin R (CI1064), etc., triphenylmethane dyes such as malachite green (CI4200), crystal violet (CI42555), methyl green (CI684), naphthalene green (CI735), etc., xanthene dyes such as rhodamine B (CI45170),

20 eosin (CI45380), fuluolesein (CI766), rose bengal (CI777), erythrosin (CI773), etc., acridine dyes such as acridine orange R (CI46005), acridine yellow (CI785), benzoflavine (CI791), acryflavine, etc., azine dyes such as safranine T (CI50240), neutral red (CI825), flavinduline O (CI824), etc., thiazine dyes such as methylene blue (CI52015), methylene green (CI924), thionine blue J (CI52025), etc., cyanine dyes such as ethyl red, quinaldine red, neocyanine, etc.,

30 styryl dyes such as 4-(p-dimethylaminostyryl), N-ethylquinolinium iodide, etc.

As a binder, those employed in usual photographic sensitive materials can be used. High molecular weight materials can be used as a binder as long as they have

35 a film-forming ability. As examples of such high molecular weight materials, there are water soluble materials such as gelatin, polyvinyl alcohol, casein, starch, hydroxyethyl cellulose, carboxymethyl cellulose, polyvinyl pyrrolidone, etc., in addition to organic solvent-soluble materials such as vinyl polymers, e.g., vinyl chloride, vinylidene chloride, vinyl acetate, etc., acrylate, polystyrene, ethyl cellulose, rubber chloride, vinylidene chloride acrylonitrile copolymer, cellulose acetate, waxes, and the like. By "High molecular weight"

40 is meant solid film-forming high molecular weight materials. The molecular weight range is 5,000 to 5,000,000, preferably 20,000 to 5 million.

45 The present invention will further be explained by the following Examples.

#### EXAMPLE 1

N-Vinylcarbazole — 1 g

Carbon tetrabromide — 0.8 g

Difurfurylidene pentaerythritol — 0.1 g

55 are dissolved in this order in 10 ml of 1,2-dichloroethane. Thereafter, a filter paper (made by TOYO KAGAKU SANGYO COMPANY, LTD., No. 4) was dipped thereinto, taken up, then dried to prepare a sensitive material. (The operation was carried out under a red safety lamp for photography. The processes of the imagewise exposure, heating, etc. are also likewise carried out. The same applies to all other Examples.) When the sensitive material thus obtained was

60 imagewise exposed to a 250 W super high pressure mercury lamp for 10 seconds at a distance of 30 cm through a photographic negative image, there was obtained a black image with a yellow background. In the

case of the combination of N-vinylcarbazole and carbon tetrabromide, the image obtained was light grayish green. By the addition of difurfurylidene pentaerythritol, the image density increased by about 0.3.

#### EXAMPLE 2

In the same manner as in Example 1 using the following furfurylidene azine instead of difurfurylidene pentaerythritol, there was prepared a light-sensitive material, which was imagewise exposed to a 250 W super high pressure mercury lamp for 10 seconds at a distance of 30 cm through photographic negative image, and then heated to 100°C to obtain a black image.



#### EXAMPLE 3

An acetone solution containing 5 g of N-vinylcarbazole was added to 50 ml of a 16 percent gelatin aqueous solution, then stirred at high speed at a temperature of 70°C for 2 minutes with the use of a homomixer (made by TOKUEHU KIKA KOGYO COMPANY, LTD.) to finely disperse the N-vinylcarbazole in the gelatin. Thereafter, dichloroethane solution containing 4 g of carbon tetrabromide and 0.5 g of difurfurylidene pentaerythritol was added thereto and emulsified and dispersed in the same manner. The resulting emulsion was coated onto a baryta paper and dried to prepare a sensitive material, which was imagewise exposed to a 250 W super high pressure mercury lamp for 10 seconds at a distance of 30 cm through a photographic negative image.

When the sensitive material was imagewise exposed to a 300 W incandescent lamp for 10 seconds at a distance of 35 cm through a photographic positive image, then the element exposed to a 250 W super high pressure mercury lamp for 10 seconds at a distance of 30 cm, there was obtained a black image thereon with pale yellow background.

#### EXAMPLE 4

N-Vinylcarbazole — 5 g  
Carbon tetrabromide — 4 g  
Difurfurylidene pentaerythritol — 0.5 g  
Crystal violet — 2 mg

were dispersed in the same manner as in Example 3 to prepare a sensitive material. The resulting sensitive material was imagewise exposed to a 300 W photographic flood lamp through a filter which transmits light of a wave length longer than 600 nm and through a photographic positive image for 10 sec. Then the element was exposed to a 250 W super high pressure mercury lamp for 10 seconds at a distance of 30 cm to obtain a black image thereon.

#### EXAMPLE 5

N-Vinylcarbazole — 5 g  
Carbon tetrabromide — 4 g  
Difurfurylidene pentaerythritol — 0.5 g  
4-(P-dimethylaminostyryl)quinoline — 1 g

were dispersed in the same way as in Example 3 to prepare a sensitive material. The resulting material was imagewise exposed to a 300 W incandescent lamp through photographic positive image for 0.5 second at

a distance of 35 cm, the whole surface thereof was then exposed to a red lamp which emits light of wavelengths longer than 600 nm for 5 seconds and finally surface thereof exposed to a 250 W mercury lamp for 10 seconds at a distance of 30 cm to obtain a black image with a pale yellow background.

#### EXAMPLE 6

Example 5 was duplicated except that polyvinyl alcohol was used instead of gelatin. After a processing as in Example 5, there was obtained a black image with a pale yellow background.

#### EXAMPLE 7

15 N-vinylcarbazole — 1 g  
Carbon tetrabromide — 0.8 g  
Difurfurylidene pentaerythritol — 0.1 g  
Dichloroethane — 2 ml

are dissolved in a 15 percent benzene solution of polystyrene. In this case, dichloroethane is used in order to dissolve the difurfurylidene pentaerythritol. The resulting solution was coated onto a baryta paper and then dried. The sensitive material thus obtained was imagewise exposed to a 250 W super high pressure mercury lamp through photographic negative image for 10 seconds at a distance of 30 cm, and was successively exposed to a 375 W infrared lamp for 30 seconds at a distance of 22 cm to obtain a black image thereon with a pale yellow background.

30 For comparison,

N-Vinylcarbazole — 1 g  
Carbon tetrabromide — 0.8 g

were dissolved in a 15 percent by weight polystyrene in benzene solution, and a photosensitive material was prepared in the same manner as in Example 7. When the resulting photosensitive material was imagewise exposed to a mercury lamp and an infrared lamp in the same way as in Example 7, there was obtained a blue image. In this case, when exposure to infrared rays was conducted for a long time, the image turned green and finally brown.

#### EXAMPLE 8

45 N-Vinylcarbazole — 1 g  
Carbon tetrabromide — 0.8 g  
Difurfurylidene pentaerythritol — 0.1 g  
Hydroquinone derivative (one of the four listed below) — 0.1 g

were dissolved in 10 ml of dichloroethane, and a photosensitive material was prepared in the same manner as in Example 1. As the hydroquinone derivatives, hydroquinone, hydroquinone monomethylether, dimethoxybenzene or P-bis(2-tetrahydropyranoyloxy) benzene were used. The photosensitive materials obtained were exposed to a 250 W mercury lamp for 5 seconds at a distance of 30 cm, then heated to 130°C. for 30 seconds to obtain a blackish-brown image thereon with a white background.

#### EXAMPLE 9

Example 8 was duplicated except that a resorcinol derivative was used instead of a hydroquinone. As the resorcinol derivatives, resorcinol, 4-ethylresorcinol, resorcinol monobenzoate or phloroglucin were used. The resulting photosensitive materials were imagewise exposed to a mercury lamp and heated in the same manner as in Example 8, and there was thus obtained a

blackish-brown image thereon with a white background.

EXAMPLE 10

N-Vinylcarbazole — 1 g  
 Carbon tetrabromide — 0.5 g  
 Hexachloroethane — 0.5 g  
 Difurfurylidene pentaerythritol — 0.1 g  
 Chloroform — 2 ml

were dissolved in 10 ml of 20 percent ethyl acetate solution of polymethyl methacrylate, a photosensitive material was prepared and processed in the same manner as in Example 7 to obtain a black image with pale polles background.

EXAMPLE 11

N-Vinylcarbazole — 1 g  
 Iodoform — 0.5 g  
 Difurfurylidene pentaerythritol — 0.1 g  
 Chloroform — 2 ml

were dispersed in gelatin to prepare a photosensitive material in the same manner as in Example 3. The resulting photosensitive material was exposed to 250 W super high pressure mercury lamp imagewise at a distance of 30 cm to obtain a black image thereon.

EXAMPLE 12

N-Vinylcarbazole — 1 g  
 Carbon tetrabromide — 0.8 g  
 Difurfurylidene pentaerythritol — 0.1 g  
 P-bis(2-tetrahydropyranoyloxy)benzene — 0.02 g  
 Dichloroethane — 2 ml

were dissolved in a 15 percent benzene solution of polystyrene, and a photosensitive material was prepared in the same manner as in Example 4. The resulting photosensitive material was imagewise exposed through a photographic negative image for 10 seconds at a distance of 30 cm, then heated to 130°C. for 5 minutes to obtain a blackish-brown image thereon with a white background. The unexposed part thereof did not color when left in a bright room.

EXAMPLE 13

N-Vinylcarbazole — 5 g  
 Carbon tetrabromide — 4 g  
 Difurfurylidene pentaerythritol — 0.5 g  
 P-bis(2-tetrahydropyranoyloxy)benzene — 0.1 g  
 4-(P-dimethylaminostyryl)quinoline — 1 mg

were dispersed in gelatin and a photosensitive material was prepared in the same way as in Example 3. The resulting photosensitive material was processed in the same manner as in Example 5 to obtain a black image thereon with pale yellow background.

What is claimed is:

1. A non-silver halide light-sensitive material for dry processing, containing the ingredients (a) polyhalogenated hydrocarbon, (b) N-vinylcarbazole and (c) furfurylidene compound; said ingredient (a) being the compound represented by the following formula:



wherein R represents H, X, COOR', or  $-C(H)_{3-n}X_n$ ; R' being a hydrogen atom, methyl group or ethyl group; X represents Cl, Br or I; and n and m represent an integer of 2 or 3; said ingredient (c) being the compound represented by the following formula:



5 wherein X represents nothing,



wherein Y and Y' are a hydrogen atom or alkyl group, for the compound represented by the following formula:



20 said ingredient (c) being present in an amount effective to increase the developed image density to blacken said image and to stabilize said image to increase its light fastness.

25 2. The non-silver halide light-sensitive material as claimed in claim 1 wherein said material further contains at least one additional compound of the ingredient (d) and ingredient (e); said ingredient (d) being hydroquinone, resorcinol or derivatives thereof, represented by the following formulas:



35 40 wherein R and R' are a hydrogen atom, an alkyl group having one to six carbon atoms, an aryl group, a hydroxyl group, a benzoyl group, an acetyl group or



45 50 , R'' represents a hydrogen atom, alkyl group having one to six carbon atoms, hydroxyl group, halogen atom or alkoxy group and n represents an integer of 1 to 4, and ingredient (e) being a photographic spectral sensitizing dye material in a dye or a dye base form.

55 5. The light-sensitive material of claim 1 wherein the ratio of the amount of ingredient (b) to that of ingredient (c) is between 100 to 1 and 1 to 100.

6. The light-sensitive material of claim 3 wherein the ratio of the amount of ingredient (b) to that of ingredient (a) is between 50 to 1 and 1 to 50.

7. The light-sensitive material of claim 2 in which the ratio of the amount of ingredient (b) to that of ingredient (d) is between 1,000 to 1 and 1 to 5 and in which the ratio of the amount of ingredient (b) to that of ingredient (e) is between  $10^5$  to 1 and 1 to 1.

8. The light-sensitive material of claim 1 further comprising a binder material.

9. The light-sensitive material of claim 6 wherein the ratio of the amount of binder material to that of the remaining ingredients of said light-sensitive material is between 1 to 100 and 20 to 1.

8. The light-sensitive material of claim 4 wherein the ratio of the amount of ingredient (b) to that of ingredient (a) is between 5 to 1 and 1 to 5 and the ratio of the amount of ingredient (b) to that of ingredient (c) is between 10 to 1 and 1 to 10.

9. The light-sensitive material of claim 5 wherein the ratio of the amount of ingredient (b) to that of ingredient (d) is between 200 to 1 and 1 to 2 and the ratio of the amount of ingredient (b) to that of ingredient (e) is between  $10^5$  to 1 and  $10^3$  to 1.

10. The light-sensitive material of claim 1 wherein said ingredient (a) is carbon tetrabromide and said ingredient (c) is difurfurylidene pentaerythritol.

11. The light-sensitive material of claim 2 wherein said ingredient (d) is P-bis (2-tetrahydropyranloxy) benzene and said ingredient (e) is 4-(p-

dimethylaminostyryl) quinoline.

12. The light-sensitive material of claim 1 wherein said ingredient (a) is capable of acting as a photoactivator which produces free radicals or ions by the action of light, said ingredient (b) is capable of reacting with said free radicals or ions produced by ingredient (a) to produce color and said ingredient (c) is capable of stabilizing and increasing the density of an image formed by the reaction of said ingredients (a) and (b).

13. The light-sensitive material of claim 2 in which R'' is an ethyl group.

14. The light-sensitive material of claim 1 in which Y and Y' represent a hydrogen atom or alkyl group having from one to six carbon atoms.

\* \* \* \* \*

20

25

30

35

40

45

50

55

60

65